

# United States Patent Office

3,532,844

Patented Oct. 6, 1970

1

3,532,844

## DISSIMILAR COMPOSITIONS FOR ELECTRICAL CONTACT PAIRS

Childress B. Gwyn, Jr., Wethersfield, Conn., assignor to Talon, Inc., Meadville, Pa., a corporation of Pennsylvania

No Drawing. Filed Oct. 26, 1967, Ser. No. 678,206  
Int. Cl. H01h 1/04

U.S. Cl. 200—166

5 Claims

### ABSTRACT OF THE DISCLOSURE

Two cooperating contacts are formed of silver cadmium and silver cadmium oxide alloys, respectively, where the silver cadmium contact is from 80 to 95% by weight silver and 5 to 20% by weight cadmium, while the other contact is from 80 to 95% by weight silver and 5 to 20% by weight cadmium oxide.

This invention relates to electrical contacts, and more particularly relates to the use of dissimilar materials for cooperating contacts.

The use of the same material for cooperating contacts is well known, and silver cadmium alloys of the same com-

position for cooperating contacts, or the use of silver cadmium oxide of the same composition for cooperating contacts is old and well known. It is also known that cooperating contacts of different composition can sometimes create improved contact service as shown, for example, in U.S. Pats. 2,300,286, 2,815,421, or 3,128,540.

In accordance with the present invention, it has been discovered that the use of silver cadmium for one of a pair of contacts, and silver cadmium oxide for the other of the pair of contacts provides unexpected and substantial improvements in the contact efficiency in regards to contact resistance, contact life, and contact arcing properties. More particularly, at least the contacting surface of one of the contacts is formed of from 80 to 95% by weight of silver

and 5 to 20% by weight of cadmium, while at least the contacting surface of the cooperating contact is formed of 80 to 95% by weight of silver and 5 to 20% by weight of cadmium oxide. The contacts can be produced in any desired manner well known to those skilled in the art, and could take any desired form such as rivets, clad surfaces, and the like.

It is, therefore, a primary object of this invention to decrease mechanical and electrical wear of cooperating contacts.

Another object of this invention is to decrease the resistance rise of a pair of cooperating contacts.

A further object of this invention is to decrease the possibility of welding in a pair of cooperating contacts.

These and other objects of this invention will become more apparent from the following examples:

A number of  $\frac{1}{4}$  inch diameter contacts were made of different compositions by standard techniques. The contacts were then arranged in a standard relay actuated by a magnet coil with a uniform contact pressure of 30 ounces. The contacts were then connected in a 220-volt 60-cycle line with a motor load (to form an inductive circuit), and the current at contact separation was measured by observation in an oscilloscope and is shown in the following chart.

| Contact composition | Peak current, amps | Type of loading | Approx. power factor, percent | Total number of operations | Approx. percent of electrical and/or mechanical wear |
|---------------------|--------------------|-----------------|-------------------------------|----------------------------|------------------------------------------------------|
| 85 Ag 15 Cd         | 140                | Motor           | 65                            | 1 130                      | 30                                                   |
| 85 Ag 15 Cd         | 140                | do              | 65                            | 2 2,600                    | 34                                                   |
| 90 Ag 10 Cd         | 151                | do              | 65                            | 1 95                       |                                                      |
| 90 Ag 10 Cd         | 151                | do              | 65                            | 2 1,265                    |                                                      |
| 85 Ag 15 CdO        | 146                | do              | 65                            | 1 425                      | 28                                                   |
| 85 Ag 15 CdO        | 146                | do              | 65                            | 2 6,000                    |                                                      |
| 85 Ag 15 CdO        | 149                | do              | 65                            | 1 4,692                    | 12                                                   |
| 90 Ag 10 Cd         | 149                | do              | 65                            | 2 19,000                   |                                                      |
| 85 Ag 15 CdO        | 153                | do              | 65                            | 1 5,409                    | 12                                                   |
| 85 Ag 15 Cd         | 153                | do              | 65                            | 2 26,000                   |                                                      |
| 90 Ag 10 CdO        | 151                | do              | 65                            | 1 2,906                    | 14                                                   |
| 95 Ag 5 Cd          | 151                | do              | 65                            | 2 16,000                   |                                                      |

<sup>1</sup> Before welding. <sup>2</sup> Before final failure.

In the above chart, the first three pairs of contact materials were of conventionally similar contact material.

The second three groups tested were, in accordance with the invention, selected of one contact of silver cadmium and the other of silver cadmium oxide. These last three pairs of materials, as shown, exhibit a dramatic improvement in number of operations to initial welding (or sticking) and to final failure (or complete welding). The consequent electrical and mechanical wear of the contact surfaces was decreased by more than 100%.

The test described above was then repeated in a resistance circuit, using a tungsten lamp load in place of the motor, using fresh contact elements. The following chart gives the result of this resistive test.

| Contact combinations | Peak current, amps | Type of loading | Power factor | Total number of operations, before welding | Approx. percent of electrical and/or mechanical erosion |
|----------------------|--------------------|-----------------|--------------|--------------------------------------------|---------------------------------------------------------|
| 85 Ag 15 Cd          | 300                | Tungsten lamps  | 1.0          | 1 1,109                                    | 38                                                      |
| 85 Ag 15 Cd          | 300                | do              | 1.0          | 2 12,234                                   |                                                         |
| 90 Ag 10 Cd          | 300                | do              | 1.0          | 1 960                                      | 40                                                      |
| 90 Ag 10 Cd          | 300                | do              | 1.0          | 2 9,300                                    |                                                         |
| 85 Ag 15 CdO         | 296                | do              | 1.0          | 1 2,908                                    | 34                                                      |
| 85 Ag 15 CdO         | 296                | do              | 1.0          | 2 10,234                                   |                                                         |
| 85 Ag 15 CdO         | 198                | do              | 1.0          | 1 4,605                                    | 16                                                      |
| 90 Ag 10 Cd          | 198                | do              | 1.0          | 2 27,009                                   |                                                         |
| 85 Ag 15 CdO         | 303                | do              | 1.0          | 1 4,808                                    | 11                                                      |
| 85 Ag 15 Cd          | 303                | do              | 1.0          | 2 31,000                                   |                                                         |
| 90 Ag 10 CdO         | 298                | do              | 1.0          | 1 3,993                                    | 20                                                      |
| 95 Ag 5 Cd           | 298                | do              | 1.0          | 2 16,240                                   |                                                         |

<sup>1</sup> Initial. <sup>2</sup> Final failure.

Again, it will be seen that the solution dissimilar materials for the contacts, in accordance with the invention, provides substantial improvement in the contact operation and life.

Although this invention has been described with respect to its preferred embodiments, it should be understood that many variations and modifications will now be obvious to those skilled in the art, and it is preferred, therefore, that the scope of the invention be limited not by the specific disclosure herein, but only by the appended claims.

The embodiments of the invention in which an exclusive privilege or property is claimed are defined as follows:

1. In combination, a pair of cooperable contacts movable into and out of engagement with respect to one another; one of said contacts having a contacting surface composed of a silver-cadmium alloy; the other of said contacts having a contacting surface composed of a silver cadmium oxide alloy; and the two contacts together providing greatly reduced susceptibility to sticking and welding, and to electrical and mechanical wear, than provided by many contact combinations of similar and other dissimilar compositions.

2. The combination of claim 1 wherein said silver cad-

mium alloy is composed of from 80 to 95% by weight silver and of from 5 to 20% by weight of cadmium.

3. The combination of claim 1 wherein said silver cadmium oxide alloy is composed of from 80 to 95% by weight silver and of from 5 to 20% by weight cadmium oxide.

4. The combination of claim 2 wherein said silver cadmium oxide alloy is composed of from 80 to 95% by weight silver and of from 5 to 20% by weight cadmium oxide.

5. The combination of claim 1 wherein said silver cadmium alloy is composed of about 85% by weight of silver and 15% by weight of cadmium and wherein said silver cadmium oxide alloy is composed of 85% by weight of silver and 15% by weight of cadmium oxide.

#### References Cited

##### UNITED STATES PATENTS

2,675,445 4/1954 Youhouse.  
2,861,155 11/1958 Farnham et al.

HERMAN O. JONES, Primary Examiner